

## UNITED STATES PATENT OFFICE

2,322,036

## CONDENSATION PRODUCT

Eugene Lieber, West New Brighton, Staten Island, N. Y., and Harry T. Rice, Roselle, N. J., assignors to Standard Oil Development Company, a corporation of Delaware

No Drawing. Application November 16, 1939,  
Serial No. 304,704

6 Claims. (Cl. 260—592)

This invention relates to novel condensation products and methods of preparing same and more particularly to condensation products which are useful as pour depressors in mineral lubricating oils.

It is known that certain fatty acid keto aromatics, or in other words ketones having the general formula  $R-CO-R'$ , in which  $R$  is an aromatic group and  $R'$  is an alkyl group having at least 10 carbon atoms, have a slight amount of pour-depressing properties. In other words, they have the characteristic of slightly reducing the pour point of waxy lubricating oils, when added thereto in small amounts such as 1% or 2%. (For measuring the pour point of an oil, the standard A. S. T. M. procedure is used.) However, such compounds are relatively weak and ineffective and have the further disadvantage of not being sufficiently soluble in mineral lubricating oils.

It is also known that when the two raw materials used for preparing such ketones, namely, aromatic hydrocarbons and an acyl halide, are reacted in such proportions as to produce a compound having two acyl groups attached to the aromatic group, the resultant diacylated aromatic compound sometimes also has some pour depressor properties, although they are not sufficiently potent in this respect to warrant commercial use, and in some cases the diacylated aromatic compound has even no pour-depressing properties.

It has now been found and is a primary object of the present invention, that by acylating an aromatic compound first to a mono-acyl stage and then continuing the acylation to the diacyl stage, the resultant product is a highly effective pour depressor. In other words, the diacylated compound made in two stages is unexpectedly much more potent as a pour depressor than the corresponding diacylated compound made in a single stage of acylation, by use of the proper proportion of the acyl halide.

For the sake of illustration, the two processes may be represented by the following two equations, of which A represents the one-stage or simultaneous acylation of the aromatic group with two acyl groups, and B represents the two-stage acylation, namely, first acylating to the mono-acyl stage and subsequently acylating to the diacyl stage:



where  $R''$  is an alkyl group of the same class as  $R'$ , but not necessarily identical therewith. It is not known why the diacylated product B should be so unexpectedly superior to the diacylated product A, although it is possible that the acyl groups in these two products are in different

positions with respect to each other around the aromatic group; for instance, in the one product the acyl group may be in ortho position and in the other case in the meta position, or even in the para position. On the other hand, it is possible that after one acyl group has already been linked to the aromatic group, the reaction which takes place upon the further addition of acyl halide may be more complicated than represented by the simple Equation B given above. In any case, however, actual test data indicate that even when starting with different types of raw material falling within the generic scope of this invention, the two-stage process is always very greatly superior to the one-stage process in respect to pour depressor properties.

Although the preparation of the mono-acyl aromatic compound is not per se within the scope of the present invention, it may be explained that one suitable method of preparing such compounds is to react a suitable aromatic compound such as benzene, naphthalene, or derivatives thereof containing inert substituents, e. g. toluene, alpha-methyl naphthalene, hexyl benzene, etc., or mixtures thereof, with the desired acyl halide, in the presence of a suitable Friedel-Crafts condensing catalyst such as aluminum chloride. The reaction usually proceeds at room temperature, and inert solvents may be used if desired. A detailed example of such a preparation will be given later.

For the preparation of the diacylated compound in a single stage or, in other words, the simultaneous combining of two acyl groups onto the aromatic group (process A), a substantially similar procedure may be used except that the amount of acyl halide used as raw material should correspond to about 2 mols of acyl halide to 1 mol of the aromatic compound; in order to insure completion of the reaction it may be necessary to heat the reaction liquid for a somewhat longer time than necessary when only acylating to the mono-acyl stage.

Similarly, in carrying out the second stage of process B, namely, the further acylation of a mono-acylated aromatic compound, the procedure used is substantially the same except that a mono-acylated aromatic compound is used as a raw material, and 1 mol of this compound is reacted with substantially 1 mol of the acyl halide to be used in combining the second acyl group onto the aromatic compound.

As a specific illustration of the invention, it has been found that when two stearyl ( $C_{17}H_{35}CO$ ) groups are simultaneously combined with a benzene molecule (process A), the resulting product produced a pour point of  $+20^{\circ} F.$  (when 2% of the addition agent was used in a waxy lubricating oil having an original pour point of  $+30^{\circ} F.$ ); on the other hand, when only one stearyl group is

combined onto a benzene nucleus, the resulting mono-stearyl benzene produced a pour point of  $+25^{\circ}$  F. (in the same lubricating oil as used above) and when, according to the present invention, that mono-stearyl benzene was further acylated to a di-stearyl benzene (process B) the product produced a pour point of  $-30^{\circ}$  F., which is vastly and unexpectedly superior to not only the mono-stearyl but also the di-stearyl benzene made by process A.

In carrying out the present invention, mono-acylated aromatic compounds having various types of aromatic groups may be used, and the invention has been found particularly applicable in the case of mono-nuclear aromatic compounds because, although a few mono-acylated aromatic compounds having rather complex polynuclear aromatic groups are fairly effective as pour depressors, yet the corresponding compounds of the simpler mono-nuclear aromatic groups are extremely weak and ineffective; and yet by the process of the present invention those weak and ineffective mono-acylated aromatic compounds may be converted into very potent pour depressors. Instead of benzene, other aromatic groups may be used such as naphthalene, diphenyl, anthracene, phenanthrene, toluene, phenol, aniline, cresol, etc.

The alkyl group R' present in the acyl group of the mono-acylated aromatic compound should have at least 10 carbon atoms and preferably at least 15 carbon atoms, such as octadecyl, heptadecyl, cetyl, etc., although some of the lower groups such as lauryl may also be used. Instead of using compounds having relatively pure alkyl groups such as those mentioned above, mixtures may be used such as the mixed fatty acids obtained from the oxidation of paraffin wax, these mixed acids being subsequently converted into the corresponding acyl halide as by treatment with phosphorus trichloride and then reacted with a suitable aromatic compound such as benzene to produce a corresponding wax-fatty acid ketone of benzene. The alkyl group of the acyl halide to be used in carrying out the second stage of the process B, namely, the primary process of the present invention, should be of the same general type as that just described, namely, having at least 10 carbon atoms and preferably at least 15 carbon atoms, but it need not be identical with the alkyl group present in the acyl group or groups already in the acylated aromatic compound.

Likewise, in carrying out the second stage of this process, a suitable Friedel-Crafts type catalyst should be used such as aluminum chloride, boron fluoride, zinc chloride, ferric chloride, titanium tetrachloride, boron chloride, anhydrous hydrogen fluoride, etc. Also, if desired, inert solvents or diluents may be used such as a kerosene or naphtha fraction, which have been highly refined by strong sulfuric acid or anhydrous aluminum chloride so as to be inert under the conditions of the present reaction. Other suitable solvents include tetrachlorethane, dichlor-benzene, or other halogenated hydrocarbon solvents or other inert liquids such as carbon disulfide, nitro-benzene, and the like.

Although obviously the amount of condensation catalyst to be used will vary to some extent according to the materials treated and according to the temperature and time of reaction, yet in general about 1 to 1.25 mols of catalyst should be used per mol of acyl chloride or halide used; this would correspond to approximately 44% to 55% <sup>75</sup>

by weight of aluminum chloride, for instance, in the case of stearyl chloride, the per cent of aluminum chloride being based on the amount of fatty acid chloride used.

5 The invention will be better understood from a consideration of the following experimental data:

Example 1.—Stearylization of mono-stearyl benzene.

The mono-stearyl ketone of benzene (phenyl 10 heptadecyl ketone) having the formula



was prepared from the following proportions of reagents:

|    |                         |                 |     |
|----|-------------------------|-----------------|-----|
| 15 | Stearic acid-----       | grams           | 350 |
|    | PCl <sub>3</sub> -----  | do              | 395 |
|    | Benzene-----            | do              | 100 |
|    | AlCl <sub>3</sub> ----- | do              | 166 |
|    | Solvent-----            | cc. of kerosene | 500 |

The stearic acid was converted to stearyl chloride by treating with the PCl<sub>3</sub> on the water bath. The resulting stearyl chloride was decanted from the phosphorous acid into a mixture of the benzene and kerosene solvents in a suitable reactor.

25 The aluminum chloride was now slowly added with suitable agitation. After the addition of the aluminum chloride, the reaction mixture was heated to about  $220^{\circ}$  F. and maintained thereat for about 5 hours. After cooling, the reaction

30 mixture was neutralized with a mixture of water and alcohol and diluted with a further 500 cc. of kerosene. After settling, the kerosene extract was distilled with fire and steam to  $600^{\circ}$  F. to remove low-boiling products (chiefly solvent and unreacted stearic acid). A yield of 362 grams of mono-stearyl ketone of benzene was obtained, consisting of a light brown wax-like solid. When 1%, 2% and 3% of the mono-stearyl ketone of benzene thus prepared, were blended in a waxy oil having a pour point of  $+30^{\circ}$  F., the pour points of the resulting blends were found to be  $+30^{\circ}$  F.,  $+25^{\circ}$  F., and  $+15^{\circ}$  F., respectively, thus showing that the mono-stearyl benzene is only relatively weak as a pour depressor.

35 45 Now, according to the present invention, some of the mono-stearyl benzene thus produced was further acylated by treatment with an additional amount of stearyl chloride in the presence of aluminum chloride, using the following amounts of materials:

|                                                       |           |                        |
|-------------------------------------------------------|-----------|------------------------|
| Mono-stearyl benzene-----                             | 344 grams |                        |
| Staryl chloride from-----                             | 284 grams | stearic acid           |
|                                                       | 77 grams  | phosphorus trichloride |
| Aluminum chloride-----                                | 138 grams |                        |
| Solvent kerosene (pretreated with AlCl <sub>3</sub> ) |           |                        |

50 55 The aluminum chloride was gradually added at room temperature and then the reaction mixture was heated to  $180$ – $200^{\circ}$  F. and maintained thereat for 4 hours, after which the catalyst was killed and the high boiling residue presumed to be essentially a di-stearyl benzene "B" was recovered from the reaction mixture (yield=503 grams), in a manner similar to that used above for the mono-stearyl benzene. The resulting di-stearyl benzene "B" when added in 2% concentration to the same waxy lubricating oil base stock having a pour point of  $+30^{\circ}$  F., as used above, reduced the pour point of the blend to  $-30^{\circ}$  F., thus showing a tremendously unexpected improvement in pour depressor properties as compared to the mono-stearyl benzene, which gave a pour point of only  $+25^{\circ}$  F. This same di-

stearyl benzene "B," when added in 1% concentration to the same oil base stock, gave a pour point of  $-20^{\circ}$  F. and when used in 1% concentration in another oil base stock having a pour point of  $+10^{\circ}$  F. gave a pour point of  $-25^{\circ}$  F.

For the sake of comparison, a di-stearyl benzene "A" was made by using the one-stage process discussed above, but using the following amounts of materials:

|                       |                                    |
|-----------------------|------------------------------------|
| Benzene               | 50 grams                           |
| Stearyl chloride from | 350 grams stearic acid<br>(2 mols) |
|                       | 100 grams $\text{PCl}_3$           |
| $\text{AlCl}_3$       | 170 grams                          |

After addition of the  $\text{AlCl}_3$  the reaction mixture was heated to  $200^{\circ}$  F. and maintained thereat for 5 hours, after which the product (yield=295 grams) considered to be essentially a di-stearyl benzene "A" was recovered from the reaction mixture in substantially the same manner as described above. This di-stearyl benzene "A" when blended in 2% concentration in the same waxy oil as used above, reduced the pour point only to  $+20^{\circ}$  F., thereby indicating that it is very weak as a pour depressor.

In other words, for some unknown reason, the di-stearyl benzene "B" of the present invention is very markedly superior to either of the known products made from the same raw materials.

*Example 2.—Acylation of benzene with paraffin wax acids.*

Another set of tests were carried out exactly the same as under Example 1, except that instead of deriving the acyl group from stearic acid it was derived from the fatty acids obtained by the oxidation of paraffin wax (cut known as #6) using an acid fraction having the following properties:

|                                |       |
|--------------------------------|-------|
| Average number of carbon atoms | 17-20 |
| Acid No.                       | 206   |
| Saponification No.             | 239   |
| Lovibond color, 6 "cell":      |       |
| Red                            | 3.0   |
| Yellow                         | 27    |

The results of this series of tests were as follows:

|                                                   | Pour point (°F.) |
|---------------------------------------------------|------------------|
| Original waxy oil                                 | +30              |
| Original waxy oil+2% mono-wax-ketone of benzene   | +5               |
| Original waxy oil+2% di-wax-ketone of benzene "A" | 0                |
| Original waxy oil+2% di-wax-ketone of benzene "B" | -35 <sup>1</sup> |

<sup>1</sup> Better than  $-35^{\circ}$  F. pour because the oil still pours freely at this temperature, but this is the lower limit of the temperatures used in the standard A. S. T. M. procedure.

Thus in both Examples 1 and 2, the product made according to the present invention by further acylation of a mono-acylated benzene gave unexpectedly superior pour depressing properties.

It will now be noted, from a consideration of the following experimental data concerning the acylation of naphthalene, that the invention is not limited to the preparation of compounds containing only two acyl groups but it can also be applied to preparation of compounds containing three or even more acyl groups and such compounds can be prepared by acylating in two or more stages. For example, tri-stearyl naphthalene can be prepared either (1) by reacting naphthalene with 2 mols of stearyl chloride and reacting the resultant di-stearyl naphthalene

"A" with another mol of stearyl chloride or (2) reacting naphthalene with 1 mol of stearyl chloride, then reacting the resultant mono-stearyl naphthalene with another mol of stearyl chloride to make a di-stearyl naphthalene "B" and finally, treating the latter with another mol of stearyl chloride. The products of either of these two processes (1) and (2) are both unexpectedly superior to a tri-stearyl naphthalene made in a single stage by treating naphthalene directly with 3 mols of stearyl chloride.

*Example 3.—Stearylization of naphthalene to di-stearyl naphthalene.*

Using the same general procedure as described under Example 1, naphthalene was treated with stearyl chloride in two stages to make di-stearyl naphthalene "B" and for sake of comparison also in one stage to make a di-stearyl naphthalene "A." Both products were tested for pour point depressing properties, along with the mono-stearyl naphthalene for comparison, using in all cases 2% of the addition agent dissolved in a waxy lubricating oil base stock having a pour point of  $+30^{\circ}$  F. The results were as follows:

|                                                   | Pour point °F. |
|---------------------------------------------------|----------------|
| Original waxy oil                                 | +30            |
| Original waxy oil + 2% mono-stearyl naphthalene   | +25            |
| Original waxy oil + 2% di-stearyl naphthalene "A" | +30            |
| Original waxy oil + 2% di-stearyl naphthalene "B" | -30            |

It is noted that whereas the di-stearyl naphthalene "A" made by direct stearylization of naphthalene in a single stage had no pour depressing properties at all, the di-stearyl naphthalene "B" made by stearylization in two stages was a powerful pour depressor, only 2% of it reducing the pour point of the waxy oil from  $+30^{\circ}$  F. to  $-30^{\circ}$  F. This also illustrates clearly how the mono-stearyl naphthalene, which is itself only an extremely weak pour depressor, can be converted by further stearylization into a very potent pour depressor.

#### Example 4

As an illustration of the application of this invention to aromatic compounds acylated to a content of 3 acyl groups, tri-stearyl naphthalene was produced by two different methods, the tri-stearyl naphthalene "A" being produced by direct stearylization of naphthalene in a single stage by using 3 mols of stearyl chloride per mol of naphthalene, and tri-stearyl naphthalene "B" being made by first stearylating naphthalene with 2 mols of stearyl chloride to make a di-stearyl naphthalene "A" and then further stearylating this product with another mol of stearyl chloride. The results of pour-depressing tests on these two compounds were as follows:

|                                                    | Pour point °F. |
|----------------------------------------------------|----------------|
| Original waxy oil                                  | +30            |
| Original waxy oil + 2% tri-stearyl naphthalene "A" | +30            |
| Original waxy oil + 2% tri-stearyl naphthalene "B" | -10            |

It is thus seen that the tri-stearyl naphthalene "B" made in two stages is far superior to the tri-stearyl naphthalene "A" made in one stage because the latter is in fact not a pour depressor at all. Furthermore, the tri-stearyl

naphthalene "B" is also far superior to the di-stearyl naphthalene "A" (made by stearylating naphthalene in one stage by using 2 mols of stearyl chloride) from which it was made because the latter had no pour-depressing properties at all.

When the product of this invention, which in effect is a wax modifier, is used as a pour depressor the amount of it to be added to a waxy lubricating oil will generally be between the limits of .01% and 10%, preferably about 0.5% to 3%, depending to a certain extent upon the amount of wax in the mineral oil and upon the degree of low temperature at which it is desired that the mineral oil be fluid.

Although it is primarily intended to use this wax modifier as a pour depressor in lubricating oils, it is also useful as an aid for settling, filtering, or centrifuging a wax, such as from a solution of hydrocarbon wax and an oil in a diluent such as naphtha, as used in dewaxing processes. For such a purpose, about 1% to 5% of the wax modifier is generally used, based upon the estimated amount of wax which is to be separated from the lubricating oil. The wax modifier of this invention is also suitable for improving the texture of wax, such as a paraffin wax, to be used for coating paper, etc., in which case the amount of wax modifier to be used should usually be within the range from about 1% to 10% in the total composition of wax and modifier.

It is not intended that this invention be limited by any theory as to the mechanism of the operation of the invention, nor by any of the specific examples which have been given merely for the

sake of illustration, but only by the appended claims in which it is intended to claim all novelty inherent in the invention as broadly as the prior art permits.

5. We claim:

1. A compound having the general formula  $R(COR')_n$  where R is an aromatic group, R' is an alkyl group having at least 10 carbon atoms and n is an integer greater than 1, said compound being

10 made by acylating the aromatic group R in at least two stages.

2. The process which comprises acylating an aromatic compound with an acyl group having more than 10 carbon atoms besides the carbon

15 atom in the CO group, to a mono-acyl derivative, and then further acylating said mono-acyl derivative with another acyl group having more than 10 carbon atoms in addition to the carbon atom in the CO group.

20 3. Process according to claim 2 in which R' has more than 15 carbon atoms.

4. The process which comprises treating a compound having the formula  $RCOR'$  in which R is an aromatic group and R' is an alkyl group

25 having at least 10 carbon atoms, with an acyl halide having the formula  $R'COX$ , in which R' is an alkyl group having at least 10 carbon atoms and X is an halogen atom.

5. A di-wax ketone of benzene made by acylation of a mono-wax ketone of benzene by a wax acid halide.

30 6. A tri-stearylated naphthalene made by stearylating naphthalene in at least two stages.

EUGENE LIEBER.  
HARRY T. RICE.